

Sept. 18, 1928.

1,684,841

J. R. C. MARSH

STEEL AND ITS MANUFACTURE

Filed Jan. 19, 1922

Fig. 1



Fig. 2



Fig. 3



Fig. 4



Witness:

F. G. Advisor.

Inventor

Joseph Russell Cornell Marsh  
By *Pame Carpenter Atty*

Patented Sept. 18, 1928.

1,684,841

# UNITED STATES PATENT OFFICE.

JOSEPH RUSSELL CORNELL MARSH, OF ARLINGTON HEIGHTS, ILLINOIS, ASSIGNOR  
TO FRANCIS NORWOOD BARD, OF CHICAGO, ILLINOIS.

## STEEL AND ITS MANUFACTURE.

Application filed January 19, 1922. Serial No. 530,261.

My present invention relates broadly to the introduction of modifying elements into metals, and more particularly to increasing the carbon content of metals such as iron and steel, and includes the introduction into the metal of a carboniferous material in such a form that it will readily combine with the metal with the introduction of the minimum of objectionable material into the resultant product and with the minimization of presence of any objectionable characteristics, and further includes the introduction of this carboniferous material in a manner that will give the most efficient results with the least deleterious incidents, with the greatest facility and accuracy.

Among the principal objects of the present invention are the production of a metal having a modifying element introduced therein, such for example as steel having a predetermined carbon content, accurately produced and reproduced on a commercial scale, a process for introducing the modifying element such as carbon during the course of production in such a manner as to gain closely predetermined results, and an improved resultant product, such as steel characterized by being within closely predetermined limits and free from objectionable characteristics.

In the accompanying drawing I have thus treated the manner in which the molten metal entrains the flaked particles of carbon preferably employed by me.

In the aforesaid drawing which I have provided for the purpose of illustrating certain steps in the carrying out of my improved method of introducing a modifying element into a metal in the manufacture, for example, of steel having a predetermined carbon content—

Figure 1 is a sectional view of a mass of flake graphite disposed in a ladle;

Figure 2 is a sectional view illustrative of the position the contents of the ladle assumes as the stream of molten metal is introduced thereinto; and

Figures 3 and 4 are views similar to those of Figures 1 and 2 illustrative of prior art to an extent desirable for the proper and adequate understanding of my present invention.

As will be understood on viewing Figures 1 and 2 of the drawing, the bottom of the ladle is indicated at 10, the mass of flake graphite at 11, the descending stream of mol-

ten metal from the furnace or cupola at 12, 55 and the mass of carburized molten metal at 13.

It will be observed on inspection of Figure 1 that the flakes of graphite lie flat in the ladle and being thin consequently quickly 60 attain the proper temperature when the ladle is properly heated.

As the stream of molten metal strikes the flakes of graphite broadside, it turns and entrains them and carries them edgewise downwardly and laterally, and inasmuch as the graphite thus entrained consists, as noted, of very thin flakes, of great superficial area which may quickly and thoroughly absorb heat, they will be readily taken up by and 70 combined with the molten metal and thoroughly disseminated throughout the mass thereof owing to the gyratory motion imparted thereto through the action of the stream 12, and thus a homogeneous product 75 is attained.

That part of the molten mass which is out of the path of the stream 12 floats upon and rises with the top of the rising mass of molten metal contained within the ladle, 10, 80 but is drawn into the mass as the stream of molten metal 12 continues to run into the ladle 11.

On comparing the illustration of Figures 1 and 2 with those of Figures 3 and 4, 85 it will be observed that when carbon in such forms as ground anthracite coal, coke breeze and the like, which is illustrated at 11<sup>a</sup>, is employed, a much greater quantity is necessary in order to have the supply of carbon of the same initial quantity as that indicated at 11.

It will be appreciated also that owing to the relatively impure form of such organic forms of carbon, the volatile matter may be 95 as much as 60% as against 2% in the case of flake graphite. It will readily be discerned that owing to the relative thickness of the particles of such organic forms of carbon not only is a much longer time required for 100 heating them, with consequent oxidization, but also when such organic forms are forced into the mass of molten metal, the volatile matter is entrained and atmospheric air is carried along in such a way as to produce 105 large and most undesirable quantities of hurtful gases such as CO, CO<sub>2</sub>, H<sub>2</sub>CO<sub>3</sub>, and the like.

In the practice of my present invention I have found it desirable for purposes of introducing carbon into metal such as in the manufacture of steel for the purpose of producing a definite carbon content combined therewith, to employ highly comminuted graphite preferably in the form of flake graphite. Such graphite is generally commercially pure in respect to sulphur, phosphorus, carborundum and the like, and is otherwise free from any detrimental content.

In the utilization of flake graphite to be introduced into the metal, as above suggested, I have found it desirable first to introduce into the ladle or other container to be used a predetermined quantity of the flake graphite which is heated and maintained in a heated state in the ladle, preferably by preheating the ladle at least to a red temperature.

The molten metal, such as steel from the furnace, is then introduced into the ladle onto the top of the heated graphite, the temperature of the mass being that required for making steel and the temperature of the graphite being such that on one hand there will be no appreciable chilling action on the metal and on the other hand all volatile or combustible matter will be expelled.

The flake graphite being lighter than the molten metal, and the flakes lying in substantially a horizontal plane, the mass thereof floats as a stratum at the top of the molten content of the ladle, thus forming a protective coating to the metal and preventing oxidation thereof, and as additional molten metal in entering the ladle passes through this stratum it not only takes up in chemical combination a portion of the carboniferous material but also initiates a quasi-circulatory movement of a physically entrained portion through the mass, thus in fact bringing the carbon and the molten metal into intimate contact in the form of a physical mixture, and so facilitating still further combination between the carbon and the molten metal, and the process may be carried on even to the point of saturation.

As a result of the use of flake graphite as a carbonaceous material two important consequences are effected which are broadly that: first, the desired chemical combination between the carbon and metal is effected to a high degree; and, second, the process may be so practiced that substantially all of the carbon may be taken into the chemical combination and the presence of free or uncombined carbon may be avoided.

By the foregoing practice the maximum contact between the particles of carbon and of molten metal is established, and as a result the maximum of chemical combination between the two is effected.

As a consequence the exact amount of carbon that will chemically combine with a predetermined amount of molten metal can be

gauged accurately in advance, and thus the manufacture of steel, for example, may be greatly facilitated.

Furthermore, in cases where it is desired to produce a chemical combination of carbon of less than the maximum, the exact amount of carbon required to produce the desired result can also be accurately gauged because of the maximum intimate contact referred to.

Conversely, in cases where it is desired to employ carbon not in chemical combination, such so-called "graphitic carbon" will be uniformly distributed through the mass, and consequently the amount of carbon necessary to result in a predetermined proportion of "graphitic carbon" throughout the mass can also be accurately gauged in advance by the employment of my improved process.

By the use of carbon in the form of flake graphite in the process described, I am enabled to obtain not only a steel having an increase of carbon content rise chemically combined of .047% but, with the same proportions between the carboniferous material and the molten mass, the desired results may be quickly, uniformly, and consistently produced.

I have thus found in actual practice that the addition of each ounce of graphite (containing 85% carbon) to each one hundred pounds of molten iron gives a rise of .048 in large quantities and .047% in small quantities, and that the maximum carbon rise has given a known and ascertained record of .85% rise made in small quantities, that is, less than one hundred pounds of steel.

For example, a .27% carbon steel has been raised by me to 1.10% carbon steel by the use of 85% flake graphite according to the process hereinabove set forth. Analysis of the carbon steel so produced showed all combined carbon and no graphitic carbon whatsoever.

Those who are skilled in the art will appreciate that not only am I able to produce for example a steel having a maximum carbon content, but also one that is simultaneously of extraordinary purity and of maximum density and homogeneity throughout owing to the expulsion of foreign and volatile matters and the prevention of the occlusion of entrained impurities and gases giving rise to hard spots, pockets and other imperfections.

Owing to the flatness and thinness characteristic of carbon particles presented in the form of the flake graphite preferably employed by me, these particles not only tend to float on the mass of molten metal in a position best adapted to be entrained by an impinging mass of molten metal but are obviously of a form most particularly adapted for instantaneous heating and as a consequence combine most quickly with the metal into contact with which they are brought as will be readily comprehended on consideration of the accompanying drawing.

The maximum chemical combination with a minimum of carboniferous material is attained where the steel making temperature is maintained during the process. Where, 5 however, this temperature is not maintained, this maximum result will not be attained, but there will occur simultaneously with the chemical combination of some of the carbon a mechanical mixture of another portion of 10 the carbon to form "graphitic carbon".

It will thus be discerned that I am enabled to produce modified ferrous materials wherein the quantity content of the modifying element, such as carbon, and also the nature 15 thereof may be regulated with great nicety and precision.

It will furthermore be manifest that because of the freedom from volatile matter, sulphur, phosphorus, carborundum and other 20 undesirable elements graphite in the form and condition employed by me, and the fact that such material does not tend to entrain atmospheric air or other gases, the practice of 25 my improved process tends neither to produce carborundum or other hard spots nor increase the amount of occluded gases in, nor the sulphur and phosphorus content of the steel thereby produced but rather to produce and enable the reproduction of a steel characterized 30 as being within closely predetermined limits, and consequently one not only free from objectionable characteristics but also one answering the desired specifications.

Having thus described my invention and 35 illustrated its use, what I claim as new and desire to secure by Letters Patent is:—

1. In the process of making steel, the steps 40 which include adding a stream of moulten metal to loose graphitic material in flake form and in a state of subdivision to be highly mobile whereby the stream of moulten metal will form an intermixed current of graphitic material and metal to rapidly and completely carburize the metal.

45 2. In the process of making steel, the steps

which include adding a stream of moulten metal to loose graphitic material in flake form, in heated condition short of ignition and in a state of subdivision to be highly mobile whereby the stream of moulten metal will 50 form an intermixed current of graphitic material and metal to rapidly and completely carburize the metal.

3. In the process of making steel, the steps 55 which include adding a stream of moulten metal to loose graphitic material in flake form and in a state of subdivision to be highly mobile and circulating the incoming stream of metal in contact with the graphitic material to have substantial portions thereof form 60 a sealing layer for the metal and continuing the circulation whereby the stream of moulten metal will form an intermixed current of graphitic material and metal to rapidly and completely carburize the metal. 65

4. In the process of making steel, the steps 70 which include adding a stream of moulten metal to loose, unconfined graphite in flake form and circulating the metal relatively to the graphite material to form intermixed currents of metal and graphite. 75

5. In the process of making steel, the steps 80 which include impinging a stream of moulten metal through a bed of unconfined flake graphite in loose form and in a state of subdivision to be highly mobile, and circulating the metal and graphite in intermixed currents while substantially maintaining the moulten metal coated with a layer of graphite. 75

6. In the process of making steel, the steps 85 which include impinging a stream of moulten metal against preheated flake graphite in a state of subdivision to be mobile and freely and completely circulate with the stream of metal and form intermixed substantially uniform currents thereof.

In testimony whereof I have hereunto signed my name.

JOSEPH RUSSELL CORNELL MARSH.